

## 1

2,892,714

## PHOTOGRAPHIC COLOR DEVELOPMENT WITH PYRAZOLINE DEVELOPERS

Ottmar Wahl, Opladen, Rudolf Mersch, Leverkusen-Bayerwerk, and Walter Püschel, Düsseldorf, Germany, assignors to AGFA Aktiengesellschaft, Leverkusen, Germany, a corporation of Germany

No Drawing. Application July 7, 1955  
Serial No. 520,608

Claims priority, application Germany July 8, 1954

2 Claims. (Cl. 96—55)

The present invention relates to a process for the production of photographic color images by color development and more especially to such processes in which 1-(4'-aminophenyl)-3-amino-pyrazolines are used as color forming developing substances.

In the production of colored images by color forming development of exposed silver halide emulsion layers, a colored image is formed in addition to the silver image by the oxidation product of the developer reacting with color couplers which are present at the same time, thereby forming a dye. Particular practical importance has formerly been assumed by those processes in which p-phenylene diamine or its derivatives have been used as developer. p-Aminophenol and its derivatives have also been described for this purpose.

It has now been found that novel effects such as were not possible with the hitherto known developers may be produced with 1-(p-aminophenyl)-3-aminopyrazoline and its derivatives in the color development of exposed silver halide emulsions. The derivatives of 1-(p-aminophenyl)-3-aminopyrazoline are obtained by substitution of the hydrogen atoms in the 1-phenyl nucleus and in the heterocyclic ring, and as substituents, there are mentioned, by way of example, alkyl, aryl, aralkyl, acyl, alkoxy, carboxy, amino, hydroxyl, halogen and sulpho groups. Examples of such compounds are: 1-(4'-amino-3'-methoxyphenyl)-3-amino-pyrazoline-dihydrochloride, 1-(4'-amino-3'-methylphenyl)-3-amino-pyrazolinedihydrochloride, 1-(4'-aminophenyl-2'-methyl)-aminopyrazoline-dihydrochloride, 1-(4'-amino-3'-oxethylphenyl)-3-amino-pyrazolinedihydrochloride, 1-(4'-amino-3'-carboxyethylphenyl)-3-amino-pyrazolinedihydrochloride.

Whereas, for example, 1-(p-aminophenyl)-4-aminopyrazolones have not been found suitable for effective color-developing, the compounds according to the present invention are compounds which have a very rapid developing and intensively color-coupling action. The color shades of the dyestuffs which are obtained by the coupling of the development products of these compounds with color couplers in color development are very different as compared with those which are obtained with the known p-phenylene diamines. As will be seen from the following Example 1, the absorption maximum of the dyestuffs obtained is displaced by up to 100 m $\mu$  to-

## 2

wards longer wave length. In addition essential differences are shown in other properties of the dyestuffs as compared with the corresponding dyestuffs obtained with the known color developers, for example, as regards increased resistance to acid. Owing to the increased developing and coupling intensity, it is possible to obtain additional advantages as regards the sensitivity of the material for color photography.

1-(p-aminophenyl)-3-aminopyrazoline may be obtained 10 by 1-(p-acylaminophenyl)-3-aminopyrazolines, such as, for example, the acetyl derivative, being subjected to alkali saponification. The derivatives of this compound may be prepared in analogous manner (see in this connection application relating to "Process for the production of 1-(p-aminophenyl)-3-aminopyrazoline" Serial No. 515,558 filed June 14, 1955, by Rudolf Mersch and Detlef Delfs, now U. S. Patent 2,840,567, granted June 24, 1958, and assigned to the assignee of the present application. Furthermore there may be applied the process disclosed in the copending application Serial No. 440,562, filed June 30, 1952, and now abandoned. Example 7 of that application discloses that the above acetyl derivative is made by introducing one mol of N-nitroso-N-(p-acetaminophenyl)-beta amino propionitrile and 200 20 grams of zinc dust into 2 liters of 10% acetic acid, after the reduction is complete filtering off the zinc slurry with suction, washing with hot acetic acid and supersaturating the filtrate with acetic acid. The 1-(p-acetyl amino phenyl)-3-aminopyrazoline precipitates out in good yield 25 and has a melting point of 204° C.

## Example 1

An exposed photographic silver halide emulsion, in which is incorporated 1-(4'-sulphophenyl)-3-palmityl-pyrazolone(5) as color coupler, was developed in a developer solution of the following composition at 18° to a gamma equal to 0.7:

|    |                                              |       |     |
|----|----------------------------------------------|-------|-----|
| 40 | 1-(p-aminophenyl)-3-aminopyrazoline chloride | g     | 0.9 |
|    | Potassium carbonate                          | g     | 70  |
|    | Potassium bromide                            | g     | 2   |
|    | Sodium sulphite                              | g     | 3   |
|    | Water                                        | litre | 1   |

The required gamma was reached after a development period of 3 minutes. The "relative sensitivity" was 2.5. Designated as "relative sensitivity"=1 in the present case is that sensitivity which is reached with a gamma equal to 0.7 with a hitherto usual developer of the following composition:

|    |                                    |       |    |
|----|------------------------------------|-------|----|
| 55 | 4-amino-ethyl-hydroxyethyl aniline | g     | 5  |
|    | Potassium carbonate                | g     | 70 |
|    | Potassium bromide                  | g     | 2  |
|    | Sodium sulphite                    | g     | 3  |
|    | Water                              | litre | 1  |

A period of 7 minutes at 18° was necessary in this developer to reach a gamma equal to 0.7.

The following table shows the color displacement produced according to the invention as compared with the color development with 4-amino-ethyl-hydroxyethyl aniline, using different color couplers:

| Color coupler                                                                   | 1-(p-Aminophenyl)-3-aminopyrazoline |                  | 4-Amino-ethoxyethyl aniline |                  |
|---------------------------------------------------------------------------------|-------------------------------------|------------------|-----------------------------|------------------|
|                                                                                 | Color                               | Absorption, Max. | Color                       | Absorption, Max. |
| <chem>C17H35CONHc2ccccc2C(=O)C(C(=O)OCC(=O)Nc3ccccc3S(=O)(=O)O)C17H35C=O</chem> | red-orange.....                     | 520              | yellow.....                 | 430              |
| <chem>C17H35CONHc2ccccc2C(=O)C(C(=O)OCC(=O)Nc3ccccc3S(=O)(=O)O)C17H35C=O</chem> | blue.....                           | 630              | purple.....                 | 530              |
| <chem>C17H35CONHc2ccccc2C(=O)C(C(=O)OCC(=O)Nc3ccccc3S(=O)(=O)O)C17H35C=O</chem> | green.....                          | 750              | blue-green.....             | 690              |
| <chem>C17H35CONHc2ccccc2C(=O)C(C(=O)OCC(=O)Nc3ccccc3S(=O)(=O)O)C17H35C=O</chem> | violet.....                         | 570              | reddish purple.             | 500              |
| <chem>C17H35CONHc2ccccc2C(=O)C(C(=O)OCC(=O)Nc3ccccc3S(=O)(=O)O)C17H35C=O</chem> | reddish ble...                      | 590              | purple.....                 | 530              |

| Color coupler                                                                  | 1(4'-Amino-3'-methoxyphenyl)-3-amino-pyrazoline |                       | 4-Amino-ethyl oxethylaniline |                       | 60 | Color coupler                                                                  | 1(4'-Amino-2'-methylphenyl)-3-amino-pyrazoline |                       | 4-Amino-ethyl oxethylaniline |                       |
|--------------------------------------------------------------------------------|-------------------------------------------------|-----------------------|------------------------------|-----------------------|----|--------------------------------------------------------------------------------|------------------------------------------------|-----------------------|------------------------------|-----------------------|
|                                                                                | Color                                           | Absorp-<br>tion, max. | Color                        | Absorp-<br>tion, max. |    |                                                                                | Color                                          | Absorp-<br>tion, max. | Color                        | Absorp-<br>tion, max. |
| <chem>C17H35C=Oc2ccccc2C(=O)C(C(=O)OCC(=O)Nc3ccccc3S(=O)(=O)O)C17H35C=O</chem> | reddish blue.                                   | 570                   | purple...                    | 530                   |    |                                                                                |                                                |                       |                              |                       |
| <chem>C17H35C=Oc2ccccc2C(=O)C(C(=O)OCC(=O)Nc3ccccc3S(=O)(=O)O)C17H35C=O</chem> |                                                 |                       |                              |                       | 65 | <chem>C17H35C=Oc2ccccc2C(=O)C(C(=O)OCC(=O)Nc3ccccc3S(=O)(=O)O)C17H35C=O</chem> | blue.....                                      | 620                   | purple...                    | 530                   |
|                                                                                |                                                 |                       |                              |                       | 70 | <chem>C17H35C=Oc2ccccc2C(=O)C(C(=O)OCC(=O)Nc3ccccc3S(=O)(=O)O)C17H35C=O</chem> |                                                |                       |                              |                       |

